

[54] DIRECTIONALLY SOLIDIFIED EUTECTIC  
TYPE ALLOYS WITH ALIGNED DELTA  
PHASE

[75] Inventors: Franklin D. Lemkey; Earl R.  
Thompson, both of Glastonbury,  
Conn.

[73] Assignee: United Aircraft Corporation, East  
Hartford, Conn.

[22] Filed: Jan. 27, 1972

[21] Appl. No.: 221,165

[52] U.S. Cl. .... 75/170, 75/171, 148/32,  
148/32.5

[51] Int. Cl. .... C22c 19/00

[58] Field of Search .... 75/170, 171; 148/32, 32.5

[56]

References Cited

UNITED STATES PATENTS

3,554,817 1/1971 Thompson ..... 148/32

Primary Examiner—Richard O. Dean  
Attorney, Agent, or Firm—Richard N. James

[57]

ABSTRACT

A nickel alloy containing columbium and/or tantalum and chromium and/or aluminum and displaying eutectic-type behavior is unidirectionally cast under conditions resulting in coupled growth, providing a lamellar biphasic or multiphasic microstructure displaying about 25–40 percent of a substantially aligned delta phase,  $\text{Ni}_3\text{Cb}$ ,  $\text{Ni}_3\text{Ta}$  or  $\text{Ni}_3(\text{Cb},\text{Ta})$ , in a nickel alloy matrix containing chromium and/or aluminum.

10 Claims, 10 Drawing Figures



PATENTED FEB 19 1974

3,793,010

SHEET 1 OF 8

**FIG.1**



**FIG.2**



PATENTED FEB 19 1974

3,793,010

SHEET 2 OF 8

FIG. 3



FIG. 5



PATENTED FEB 19 1974

3,793,010

SHEET 3 OF 8

FIG. 4



PATENTED FEB 19 1974

3,793.010

SHEET 4 OF 8

FIG. 6



PATENTED FEB 19 1974

3,793,010

SHEET 5 OF 8

FIG. 7

— SINGLE PHASE FIELD BOUNDARY  
--- EUTECTIC TROUGH



PATENTED FEB 19 1974

3,793,010

SHEET 6 OF 8

POLYHERMAL PROJECTION SHOWING BIVARIANT  
EUTECTIC SURFACE WHEREIN  $\rightleftharpoons \delta + \delta'$

FIG. 8



## INTERRUPTED OXIDATION OF Ni-Cb-Cr-Al ALLOYS (2000°F)

FIG. 9





## DIRECTIONALLY SOLIDIFIED EUTECTIC TYPE ALLOYS WITH ALIGNED DELTA PHASE

### BACKGROUND OF THE INVENTION

The present invention relates to anisotropic castings resultant from the unidirectional solidification of nickel-(columbium, tantalum)-(chromium, aluminum) eutectic-type alloys.

It is now known that certain eutectic alloys respond to proper unidirectional solidification techniques to produce useful phase-aligned microstructures, as described in the patent to Kraft U.S. Pat. No. 3,124,452. In the patent to Thompson U.S. Pat. No. 3,554,817, there is described a particularly promising pseudo-binary eutectic alloy occurring between the intermetallic compounds  $\text{Ni}_3\text{Al}$  and  $\text{Ni}_3\text{Cb}$  which responds to plane-front solidification producing a casting characterized by an aligned lamellar microstructure. As so cast, this combination provides the strongest nickel-base alloy known. As is the case with most nickel-base alloys, however, improvements in the oxidation resistance are desired, particularly to permit maximum utilization of the strength characteristics of the alloy in the very high temperature ranges. And even though in its usual application a given alloy may be provided with surface protection for increased oxidation-erosion resistance, improvements in corrosion resistance in the underlying substrate are nevertheless desirable.

In a prior patent of the same inventors, Thompson and Lemkey U.S. Pat. No. 3,564,940, there is described a class of compositions which solidify according to the monovariant eutectic reaction, providing aligned polyphase structures, including such systems as the ternary alloys identified as cobalt-chromium-carbon and nickel-aluminum-chromium. The advantage of compositions of this nature is that the desired microstructure can be achieved over a range of compositions within a given system. This provides a substantial increase in the freedom of selection of composition permitting increased optimization of properties. In a copending application of the same inventors filed Dec. 10, 1969, application Ser. No. 883,713, now U.S. Pat. No. 3,671,223, the concept has been further developed to include those systems solidifying according to the multivariant eutectic reaction where two or more solid phases ( $n$ ) crystallize simultaneously from a liquid consisting of ( $n+2$ ) or more components.

### SUMMARY OF THE INVENTION

The present invention relates to eutectic-type alloys within a basic nickel-(columbium, tantalum)-(chromium, aluminum) system which respond to plane-front solidification to provide phase-aligned microstructures comprising a lamellar delta phase in a nickel alloy matrix. As directionally solidified, these alloys are characterized by a nickel alloy matrix containing up to about 35 weight percent chromium and/or up to about 4 weight percent aluminum in solid solution and about 25-40 volume percent of a lamellar  $\text{Ni}_3\text{Cb}$ ,  $\text{Ni}_3\text{Ta}$  or  $\text{Ni}_3(\text{Cb},\text{Ta})$  delta phase in alignment therein.

In a preferred composition the alloy, as directionally cast, is nominally characterized by a nickel-chromium-aluminum matrix phase containing up to about 35 weight percent chromium and up to about 4 weight percent aluminum in solid solution with about 25-40

volume percent of the lamellar delta ( $\delta$ ) phase in alignment therein. In a particular preferred embodiment, the as directionally cast alloy is age hardenable through the precipitation of  $\gamma'$  (a phase based on the intermetallic compound  $\text{Ni}_3\text{Al}$ ) as a dispersed phase in the  $\gamma$  matrix.

### BRIEF DESCRIPTION OF THE DRAWINGS

FIG. 1 is a photomicrograph of a longitudinal section 10 of a directionally solidified alloy of the present invention at the monovariant eutectic composition comprising, by weight, 73 percent nickel, 21 percent columbium, and 6 percent chromium (200  $\times$  before reduction).

15 FIG. 2 is a similar photomicrograph of another directionally solidified alloy at the monovariant eutectic composition comprising, by weight, 71 percent nickel, 20 percent columbium, and 9 percent chromium.

20 FIG. 3 is a photomicrograph of a longitudinal section 20 of a directionally solidified alloy of the present invention at the monovariant eutectic composition comprising, by weight, 76.4 percent nickel, 20.8 percent columbium, and 2.8 percent aluminum.

25 FIG. 4 is a photomicrograph of a transverse section 25 of a bivariant eutectic composition from the  $\text{Ni}-\text{Cb}-\text{Cr}-\text{Al}$  system wherein  $\gamma'$  phase precipitation has occurred.

30 FIG. 5 is a photomicrograph of a longitudinal section 30 of an alloy at the composition comprising, by weight, 60 percent nickel, 30 percent tantalum and 10 percent chromium, as directionally solidified.

35 FIG. 6 is a graph comprising the liquidus properties 35 in the nickel-columbium-chromium system.

FIG. 7 is a graph showing the eutectic troughs and 40 single phase field boundaries in the nickel-rich corner of the nickel-columbium-aluminum diagram.

45 FIG. 8 is a representation showing a polythermal projection of the nickel-columbium-chromium-aluminum diagram which illustrates the bivariant surface wherein the three-phase equilibrium of the type  $\text{L} \gamma + \delta$  occurs.

50 FIG. 9 is a graph demonstrating the response of a  $\gamma + \delta$  monovariant eutectic alloy and a  $\gamma + \delta$  bivariant eutectic alloy to cyclic furnace oxidation at 2,000°F, as 45 compared to certain other alloy systems.

55 FIG. 10 is a graph comparing the sulfidation erosion 55 resistance of a bivariant nickel-columbium-chromium-aluminum alloy with other high temperature alloys.

### DESCRIPTION OF THE PREFERRED EMBODIMENTS

As previously described, the articles to which the present invention has reference are the directionally solidified alloy castings of monovariant or multivariant eutectic composition which display about 25-40 volume percent of an aligned lamellar  $\delta$  phase embedded in a  $\gamma$  matrix. The  $\delta$  phase includes not only the  $\text{Ni}_3\text{Cb}$  and  $\text{Ni}_3\text{Ta}$  intermetallic but also, where both columbium and tantalum are present, include the phase represented as  $\text{Ni}_3(\text{Cb},\text{Ta})$ .

The  $\gamma$  phase is a nickel-base alloy containing chromium and/or aluminum, preferably both. This phase may contain up to about 35 weight percent chromium and up to about 4 weight percent aluminum in solid solution as cast. In a preferred embodiment, the matrix will also display, upon aging, a cuboidal  $\gamma'$  phase strengthening precipitate together with, in some cases,

a disc-shaped phase which is believed to be the  $\gamma''$  phase, a tetragonal compound of nickel and columbium.

The  $\delta$  phase alignment in these alloys is clearly shown in FIGS. 1-5. FIGS. 1-3 and 5 show various articles of monovariant ternary eutectic composition as directionally solidified. FIG. 4 is a quaternary nickel-columbium-chromium-aluminum alloy, a preferred embodiment exhibiting bivariant eutectic behavior in solidification. Particular note will be taken in FIG. 4 of the strengthening cuboidal  $\gamma'$  precipitate in the matrix phase.

The articles thus described are those achieved by unidirectional solidification of alloys in the nickel-(columbium, tantalum)-(chromium, aluminum) compositional system exhibiting monovariant or multivariant behavior upon solidification with an aligned  $\delta$  phase. In this compositional system, the columbium and tantalum appear, generally speaking, to be broadly mutually substitutional or essentially an atomic basis. Either chromium or aluminum or both may be present in the alloy, providing up to about 35 weight percent chromium and up to about 4 weight percent aluminum in the matrix phase as cast.

The general compositional limitations in terms of the melt can best be ascertained by reference to FIGS. 6-8. FIG. 6 details the liquidus properties in the nickel-columbium-chromium ternary system while FIG. 7 illustrates the eutectic troughs and single phase field boundaries in the nickel-rich corner of the nickel-columbium-aluminum diagram.

The compositions in the quaternary nickel-columbium-chromium-aluminum alloy system of this invention solidify according to the bivariant eutectic reaction, which describes the compositions, defined by a liquidus surface, wherein two solid phases separate from the liquid upon solidification.

Referring to FIG. 8, this surface (shaded in the drawing) will be seen to be bounded by eutectic troughs extending, in the nickel-columbium-chromium system between but exclusive of the binary eutectic Ni— $Ni_3Cb$  and the ternary eutectic Ni— $CbCr_2$ — $Ni_3Cb$ , and, in the nickel-columbium-aluminum system, between but exclusive of the binary eutectic Ni— $Ni_3Cb$  and the ternary eutectic Ni— $Ni_3Al$ — $Ni_3Cb$ .

Compositions on the monovariant eutectic troughs have been found to provide the desired phase alignment and characteristic properties. The aligned longitudinal microstructures of the compositions comprising, by weight, 73 percent nickel, 21 percent columbium (297C), and 6 percent chromium, and 71 percent nickel, 20 percent columbium (109C), and 9 percent chromium are shown in FIGS. 1 and 2, respectively. The aligned longitudinal microstructure of a composition comprising, by weight, 76.4 percent nickel, 20.8 percent columbium, and 2.8 percent aluminum, is shown in FIG. 3. That of the alloy comprising, by weight, 60 percent nickel, 30 percent tantalum and 10 percent chromium in longitudinal section is seen in FIG. 5. The  $\delta$  phase is  $Ni_3Ta$  and the  $\gamma$  phase is a solid solution of nickel and chromium.

The transverse microstructure of the quaternary alloy comprising by weight, 68 percent nickel, 20.6 percent columbium, 9.2 percent chromium and 2.2 percent aluminum, as shown in FIG. 4, provides clear evidence of the maintenance of the physical aspects of the desired lamellar microstructure. Within the  $\gamma$  ma-

trix there are seen precipitates of both a cuboidal  $\gamma'$ , an intermetallic compound based on  $Ni_3Al$ , and a disc-shaped phase which is believed to be  $\gamma''$  frequently observed in the superalloys containing significant amounts of both aluminum and columbium. As will be noted, the lamellar  $Ni_3Cb$ ( $\delta$ ) phase comprises approximately 30 volume percent of the microstructure.

Unidirectionally solidified articles of the Alloy 297C composition, when tested in the direction of phase alignment at both room temperature and at 2,000°F, have demonstrated significant strengthening attributable to the aligned microduplex structure. This alloy has exhibited a tensile strength of 171,000 psi at room temperature. The strengths of this alloy solidified at 2 cm/hr and 10 cm/hr were at 2,000°F, respectively, 60,200 psi with a failure strain of 6 percent, and 74,400 psi with a failure strain of 8.5 percent. These values of tensile strength approach those reported for the nickel-columbium-aluminum eutectic system of U.S. Pat. No. 3,554,817, supra, and represent a significant strength increase over the conventional nickel-base superalloy systems. In addition, as hereinafter described in greater detail, additional increases in strength and ductility are attainable by suitable alloy modification within the basic bivariant or multivariant alloy solidification mechanism.

In the nickel-chromium type alloys, the corrosion resistance in oxidizing atmospheres is strongly or primarily dependent upon the chromium content of the system. Since oxidation of these alloys, as represented by the scaling rate, exhibits a minimum in corrosion susceptibility as the chromium content is varied, biphase alloys in the nickel-chromium-columbium system of a composition defined by the monovariant eutectic trough may be selected to provide the maximum oxidation resistance for a given environment. This flexibility in composition adjustment is inherent in the present invention.

Similarly, aluminum is recognized to act beneficially in increasing oxidation resistance of castings. Thus, chromium and aluminum separately as in the nickel-columbium-chromium and nickel-columbium-aluminum alloys, respectively, or in combination as in the nickel-columbium-chromium-aluminum alloys may significantly improve the oxidation properties.

The oxidation properties of eutectic alloys at compositions comprising, by weight, 69 percent nickel, 19 percent columbium, 12 percent chromium having a matrix composition ( $\gamma$ ) of, by weight, 66 percent nickel, 27 percent chromium, and 7 percent columbium, and 69.9 percent nickel, 20.4 percent columbium, 9.2 percent chromium, 0.5 percent aluminum were ascertained at 2,000°F. The results are graphically illustrated in FIG. 9. These alloys are demonstrably superior in terms of their oxidation resistance to both the Ni— $Ni_3Cb$  and Ni<sub>3</sub>Al— $Ni_3Cb$  eutectic alloys, and compare favorably with the conventional nickel-base superalloys of high corrosion resistance.

The results of a burner ring thermal cycle test on an alloy test bar at the composition comprising, by weight, 69.7 percent nickel, 20.2 percent columbium, 9.1 percent chromium, and 1.0 percent aluminum together with various other nickel-base superalloys is shown in FIG. 10. The specimens in this test were held in cycles of 1,750°F for three minutes followed by heating to 2,050°F for two minutes and cooling to 600°F while rotating in a jet burner using JP-5R fuel with 3.5 ppm sny-

thetic sea salt operating at Mach 0.3. Besides the excellent relative ranking of the alloy from this test, of as great an interest was the fact that the material suffered no decrease in tensile properties after 219.5 hours of thermal cycling. After vane cyclic sulfidation testing the erosion bar was machined into a tensile specimen such that the area of greatest erosion was within the gage length and tested at 2,000°F in air at a strain rate of 0.02 per minute. The ultimate tensile strength and strain to failure were 53,400 psi and 14.2 percent respectively while the strength and failure strain were 52,500 psi and 17.9 percent prior to rig testing.

Alloys in the system of the present invention are tolerant of the selected addition of other materials to the basic ternary and quaternary compositions. In general, deviations from or additions to the composition loci defining the monovariant and bivariant eutectic reaction may be made providing, however, that in kind and quantity they do not interfere with the basic coupled growth mechanism by which the lamellar biphase microstructure is produced. In this respect, the eutectic-type alloys, in general, have been found to be tolerant of the addition of sometimes rather substantial quantities of other elements, usually selected to provide or promote the development of a particular property or characteristic in the casting.

A number of ingredients are known to have a profound effect on alloy properties, even though present only in very small amounts. Yttrium and the rare earth elements, for example, in quantities as low as 0.03 weight percent, have been found to promote oxide adherence to the nickel-base superalloys. In some cases, quantities of boron, carbon, hafnium and zirconium have been found to promote creep rupture ductility and, in some cases, cause a pronounced reduction of the tendency of such materials to grain boundary oxidation. As previously mentioned, however, those modifications to the basic ternary or quaternary alloys which provide advantageous results and do not interfere with the development of the desired lamellar microstructure may be included therein. Generally, the solidification rates, typically about 0.5-10 cm/hr, usually associated with the unidirectional solidification of the eutectic-type alloys are also applicable to the present invention. The greater degree of dispersed phase alignment normally occurs in the case of solidification from the ideally planar liquid-solid interface. However, a substantial and, obviously in many cases, satisfactory phase alignment is also achieved from the cusped interface which may occur at the higher solidification rates.

Accordingly, the invention in its broader aspects is not limited to the specific methods, compositions and examples herein described, but numerous modifications, alterations and additions may be made thereto without departing from the true spirit of the invention and without sacrificing its chief advantages.

We claim:

1. A directionally solidified alloy casting having an overall composition selected from the group consisting of the monovariant and multivariant eutectic nickel-base alloys solidifying in a polyphase structure consisting of, a  $\delta$  phase of the  $\text{Ni}_3\text{M}$  type where M represents at least one element selected from the group consisting of columbium and tantalum and a  $\gamma$  phase consisting of a nickel-base alloy containing at least one element selected from the group consisting of chromium and aluminum, and characterized by an anisotropic microstructure having the  $\delta$  phase solidified as lamellae in substantial alignment in a matrix consisting essentially of the  $\gamma$  phase.

2. A casting according to claim 1 wherein: the  $\delta$  phase comprises about 25-40 volume percent of the casting.

3. A casting according to claim 1 wherein: the  $\gamma$  phase is a nickel-base alloy containing at least one element selected from the group consisting of chromium and aluminum in an amount of, as cast, not exceeding, by weight, about 35 percent chromium and about 4 percent aluminum.

4. A casting according to claim 3 wherein: the  $\gamma$  phase contains both chromium and aluminum and the  $\gamma$  phase, as aged, contains a fine  $\gamma'$  strengthening phase precipitate.

5. A directionally solidified alloy casting of substantially monovariant eutectic composition characterized by an anisotropic microstructure having a lamellar  $\text{Ni}_3\text{Cb}$  phase substantially aligned in a nickel-base alloy matrix containing in solid solution an element selected from the group consisting of chromium and aluminum.

6. A casting as in claim 5 wherein: the  $\text{Ni}_3\text{Cb}$  phase occupies about 25-40 volume percent of the casting.

7. A directionally solidified alloy casting of substantially monovariant eutectic composition characterized by an anisotropic microstructure having a lamellar  $\text{Ni}_3\text{Ta}$  phase substantially aligned in a nickel-base alloy matrix containing in solid solution an element selected from group consisting of chromium and aluminum.

8. A casting as in claim 7 wherein: the  $\text{Ni}_3\text{Ta}$  phase occupies about 25-40 volume percent of the casting.

9. A directionally solidified alloy casting of substantially multivariant eutectic composition characterized by an anisotropic microstructure having about 25-40 volume percent of a lamellar  $\text{Ni}_3\text{M}$  phase, where M is selected from the group consisting of tantalum and columbium, embedded in substantial alignment in a nickel-base alloy matrix containing in solid solution as cast up to 35 weight percent chromium and up to about 4 weight percent aluminum.

10. A casting according to claim 9 wherein: the matrix phase also contains fine particles of a strengthening  $\gamma'$  precipitate.

\* \* \* \* \*